

April 18, 1933.

N. R. CAMPBELL

1,904,895

MANUFACTURE OF PHOTO ELECTRIC CATHODES

Filed Dec. 16, 1930



Inventor.  
Norman R. Campbell  
M. H. Lockwood  
Attorney.

## UNITED STATES PATENT OFFICE

NORMAN ROBERT CAMPBELL, OF WATFORD, ENGLAND, ASSIGNOR TO THE GENERAL ELECTRIC COMPANY LIMITED, OF LONDON, ENGLAND

## MANUFACTURE OF PHOTO-ELECTRIC CATHODES

Application filed December 16, 1930, Serial No. 502,639, and in Great Britain January 6, 1930.

This invention relates to the manufacture of photoelectric cathodes of the type produced by the deposition of a highly electro-positive metal on a support coated with a compound with which that metal reacts chemically.

Photoelectric cathodes are known consisting of a thin film of an alkali or alkaline earth metal deposited on an oxidized surface of another metal, such as copper or silver. In one known process of preparing such cathodes, there are three distinct stages. In the first stage the underlying metal is oxidized; in the second, the alkali metal is introduced into the tube containing the cathode; in the third, the cathode, and usually the whole of the tube containing it, are baked. During this third stage, some reaction takes place between the alkali metal and its support; and, if there is any alkali metal remaining in excess after this reaction, it is driven from the cathode, and usually out of the tube.

The properties of the cathode produced by this process depend in some measure on the quantity of the electropositive metal introduced during the second stage. The facts have been explored most thoroughly when the alkali metal is caesium and the underlying metal silver; it will be convenient to describe the invention with reference to this example. If the quantity is less than a certain limit, depending on the area of the cathode as well as on other factors, the surface of the cathode becomes relatively dark in the third stage and no excess of caesium appears; this state of the cathode will be called A. If the quantity is greater than this limit, the colour of the cathode is considerably lighter after the third stage and excess caesium appears; this state will be called B. In state A the photoelectric emission increases in general with the amount of caesium introduced; but in state B it may decrease with the amount introduced. There is thus an optimum amount of caesium that should be introduced in the second stage, corresponding roughly to the limits between the amounts that lead to states A and B.

But I have found that the photoelectric emission depends not only on the amount of

caesium introduced, but also on the rate at which it is introduced and on the temperature of the cathode support during its introduction. The best results are obtained by combining the second and third stages, so that the caesium is introduced slowly while the cathode support is hot. A convenient way of effecting this is to have the caesium in a side vessel connected to the tube through a constriction and to maintain both the tube and the caesium container at a temperature of about 200° C., so that the caesium vapour distils slowly through the constriction into the tube containing the hot cathode.

According to the first feature of the invention, in the manufacture of photoelectric cathodes of the type described, the cathode support on which the cathode is to be formed is maintained at a temperature considerably above 50° C. while the vapour of the electro-positive metal is brought into contact with it in a stream considerably slower than would be obtained if that metal were maintained at the temperature of the cathode and in its immediate neighbourhood in a vacuum.

In carrying out the process according to the invention it is necessary to stop the supply of caesium when the optimum amount has been introduced. There are two obvious ways of doing this. One is to limit the amount of caesium originally present to the optimum amount; another is to stop the process at intervals and test the photoelectric emission. Neither of these is convenient. The first is inconvenient because the accurate control of small amounts of caesium is difficult, and also because the exact amount of caesium required cannot always be foretold since it varies with variations in the preceding parts of the process. The second is slow and cumbrous. I have found that a much better method is based on the observation of the thermionic emission from the cathode. At the temperature at which the cathode is maintained, it has an appreciable thermionic emission, which can be readily measured while the process is going on. This emission increases in general so long as the cathode is in state A and less than the optimum amount of caesium has been introduced; when the

limit between states A and B has been reached, the thermionic emission decreases suddenly. Accordingly in order to determine when the optimum amount has been introduced, it is only necessary to watch the change of thermionic emission; as soon as the gradual rise stops and is followed by a rapid fall, the oven is removed and the supply of caesium stopped by sealing off the caesium container at the constriction. Immediately after this operation is performed, the photoelectric emission is comparatively small. If the baking at 200° C. is now continued with the caesium container removed, the thermionic and the photoelectric emissions increase once more and the latter gradually attains a maximum not greatly altered by further baking. The process can therefore be completed by baking for a period known to be long enough for this maximum to be attained. No further watching is required.

According to the second feature of the invention, the point at which the slow stream of electropositive metal should be stopped is determined by observation of the thermionic emission of the cathode.

I have used the term thermionic emission in this description. The current that flows between the electrodes during the introduction of the electropositive metal into the hot tube resembles a true thermionic emission from the cathode in that it increases rapidly with the temperature and can be saturated by a sufficiently large potential. But I do not commit myself to the view that it is a true thermionic current dependent only on the temperature and surface of the cathode; it is possible that it consists, wholly or in part, of ions or electrons generated by the chemical reaction proceeding.

One example of the process according to the invention will now be described with reference to the accompanying drawing. The photoelectric tube is of an ordinary type, consisting of a cylindrical glass vessel *a* 40 millimetres in diameter and 80 millimetres long, on the inside wall of which silver has been deposited chemically, leaving a window *b* for the entry of light and a bare portion *c* for insulation around the anode lead. The cathode lead is a wire *d* sealed through the wall of the vessel and making contact with the silver coating; the anode is a wire frame *e* or a rod supported axially in the vessel by its lead *f* which passes out through one end. Alternatively the cathode may be a silver plate supported in the tube and the anode a gauze surrounding it; indeed any of the familiar types of tube may be used. The vessel is provided with two side tubes, one of which *g* leads to the exhaust pump and the other *h* is a tube parallel to the axis of the vessel and a few millimetres distant from it. The bottom of this second tube *h* is sealed

off, several centimetres below the bottom of the vessel *a*, and contains initially a small quantity of caesium azide. Both tubes *g*, *h* are constricted where they join the vessel *a*, the constriction *k* in the tube *h* containing the caesium azide being somewhat longer and preferably narrower than the constriction such as *m* usually made for the purpose of sealing off.

The vessel is baked and exhausted in the usual manner; during this process the bottom of the tube containing caesium azide should project from the oven and should not be allowed to reach a temperature much exceeding 300° C. The silver coating is then superficially oxidized. The oxidation may be effected conveniently in a known manner by filling the vessel with oxygen to a pressure of one millimetre and passing an electric glow discharge through the vessel with the silver coating as cathode. The coating changes colour as it oxidizes, and the oxidation may be stopped at an appropriate stage when the right colour, determined by trial, has been attained. Considerable latitude is permissible; but I have found a deep blue colour to be suitable. The oxygen is pumped out and the caesium azide decomposed by heating the tube, so that caesium is liberated. With the exhaust pump always in action the oven is lowered again at a temperature of about 200° C.; it is dangerous to exceed 220° C., but lower temperatures than 200° C. merely prolong the process. The electrodes of the tube are connected in series with a galvanometer or microammeter and a source of about 20 volts, the silver coating being negative. After a minute or two a current is indicated, and increases till it reaches a maximum which is usually in the neighbourhood of 50 microamperes after a time of the order of 10 minutes, but depending greatly on the size of the constriction through which the caesium vapour enters. After the maximum the current decreases very rapidly; it may fall to a small fraction of a microampere; or it may fall and then rise again rapidly, being now unsaturated and obeying Ohm's law. This unsaturated current is carried by a film of excess caesium bridging the insulation. Again the current having reached a first maximum may fall slowly and slightly and then rise slowly to a second and higher maximum from which the rapid fall takes place. The changes of the current may vary considerably; but the rapid fall, either to almost zero or to a current that is definitely unsaturated, can always be detected. As soon as this fall has certainly started, the temperature is raised and the caesium tube sealed off. The temperature is then lowered again for about half an hour to remove the excess caesium. Finally the tube may be filled with a rare gas, sensitized and sealed off.

What I claim is:—

1. In the manufacture of a photoelectric cathode, the process which comprises heating a support, coated with a compound that is to react with an electropositive metal, to a temperature above 50° C., producing a slow stream of the vapour of the electropositive metal, bringing the said stream into contact with the said support, measuring the space current between the support and the anode of the photoelectric tube during the passage of the said stream and stopping the stream when the said space current diminishes rapidly. 70
2. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., producing a slow stream of the vapour of the electropositive metal and bringing the said vapour into contact with the said surface layer while the said electrode is maintained at said temperature exceeding 50° C. 75
3. In the manufacture of a photoelectric cathode the process which comprises taking a tube and forming on the electrode that is to become the cathode a surface layer consisting of a compound that reacts with the electropositive metal that is to be introduced, said tube containing the said electrode being connected to a vessel containing the electropositive metal through a tube of small cross section, then heating both the tube and the vessel to a temperature exceeding 50° C., and maintaining said temperature so that a slow stream of the vapour of the electropositive metal passes from said vessel to said tube and is brought into contact with said surface layer. 80
4. In the manufacture of a photoelectric cathode the process which comprises forming on the electrode that is to become the cathode a surface layer consisting of a compound that reacts with the electropositive metal that is to be introduced, heating said electrode to a temperature exceeding 50° C., producing a slow stream of the vapour of the electropositive metal and bringing the said vapour into contact with the said surface layer while the said electrode is maintained at said temperature exceeding 50° C., and stopping the stream when the optimum amount of vapour of the electropositive metal has been introduced into the neighborhood of the said support. 85
5. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 90
6. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 95
7. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 100
8. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 105
9. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 110
10. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 115
11. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 120
12. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 125
13. In the manufacture of a photoelectric cathode, the process which comprises forming on the electrode that is to become the cathode a surface layer consisting of a compound that reacts with the electropositive metal that is to be introduced, heating said electrode to a temperature exceeding 50° C., 130